

## UNITED STATES PATENT OFFICE

2,444,022

PROCESS OF MAKING A SOLUTION  
OF CELLULOSEAart Buurman, Velp, Netherlands, assignor to  
American Enka Corporation, Enka, N. C., a  
corporation of DelawareNo Drawing. Application September 30, 1946,  
Serial No. 700,354. In Germany June 27, 1941Section 1, Public Law 690, August 8, 1946  
Patent expires June 27, 1961

11 Claims. (Cl. 106—203)

1

The present invention relates to the manufacture of cellulosic solutions to be employed in the production of threads, filaments, films and the like, and more particularly to a method of preparing alkali metal salt solutions of soda cellulose, sulphite cellulose, or cotton linters, etc., hereinafter generically referred to as cellulose.

It is known to manufacture artificial products from alkaline solutions of sodium zincate or sodium stannate, having cellulose dissolved therein. There are several methods of preparing these solutions, e. g., the cellulose is first heated to a temperature of about 115° C. and then cut up and finally dissolved at a temperature of about 0° C. The cellulose can also be chemically degraded by treatment with bisulphite solutions under pressure or by treatment with dilute sodium hydroxide followed by a substantial ripening. Such degraded cellulose can then be dissolved in solutions of sodium zincate or sodium stannate by cooling the mixture to 0° C. or below, and maintaining this low temperature until complete dissolution of the cellulose fibers, whereupon the solutions are warmed up quickly to room temperature and formed into artificial products.

The present invention contemplates a process of forming cellulosic solutions of an alkaline metal salt wherein it is unnecessary to degrade the cellulose by prolonged treatment with bisulphite solutions under pressure or by treatment with the dilute sodium hydroxide solution followed by ripening.

It is a further object of the invention to introduce normal cellulose, i. e., soda cellulose, sulphite cellulose, or cotton linters, immediately into a dilute alkaline solution of sodium zincate or sodium stannate containing an oxidizing agent.

In the preparation of the solution, an oxidizing agent such as hydrogen peroxide is first mixed with a dilute solution of sodium zincate or sodium stannate, and uniformly cut up cellulose is introduced with stirring. The mixture forms a thick pulp which is left standing until the desired degree of degradation of the cellulose is reached. Then the known procedure is followed, namely, the pulp is cooled down to below 0° C. with the result that the cellulose dissolves, and the solution is then quickly warmed up to about room temperature and is in readiness for spinning into threads, films, and the like.

During the preparation of the solution, if any excess of oxidizing agent is present, suitable chemicals, for example, a reducing agent such as formaldehyde may be added so as to prevent further degradation of the cellulose. The form-

2

aldehyde may be added to the solution either before cooling the cellulose pulp or at a later stage in the process. The time required for the degradation of the cellulose can also be regulated by utilizing a constant temperature at which the degradation takes place, or by using catalysts or by both fixing the temperature and using a catalyst.

It can be readily seen that the present invention represents a substantial simplification of the known methods of preparing these types of solutions wherein both the old and the new methods degrade the cellulose to a measured extent prior to the formation of the solution. It is a substantial saving to eliminate the prolonged treatments of cellulose with bisulphite solutions at high temperatures and under pressure, or treatments with dilute sodium hydroxide, which in turn necessitates dipping, pressing and cutting up of the cellulose fibers. In contra-distinction, the cellulose is immediately introduced into a dilute alkaline solution of sodium zincate or sodium stannate which has previously been mixed with an oxidizing agent. Thus, by allowing the pulp to age in this condition, an oxidizing degradation of the cellulose takes place.

## Example 1

3350 gms. of sodium zincate solution at 25° C. containing 9.3% NaOH and 2.3% Zn, was mixed with 330 gms. hydrogen peroxide (3%) and the mixture was thoroughly stirred. 320 gms. of cut up sulphite cellulose with a moisture content of 10% was added to this solution under constant stirring. A thick pulp formed which was left standing for 48 hours at 25° C., whereafter the pulp was cooled down to -7° C. resulting in dissolution of the cellulose. The solution was then warmed up to 16° C. and was in proper condition for spinning. Further degradation of the cellulose by an excess of hydrogen peroxide was prevented by adding 5 cm<sup>3</sup> of formaldehyde. The spinning solution obtained in this manner was stable and easily spinnable.

## Example 2

20 mg. of nickel sulphate was added to 3650 gms. of sodium zincate solution containing 8 1/2% NaOH and 2.1% Zn. at 24° C., after which 30 gms. of 30% hydrogen peroxide was added. 320 gms. of cut up sulphite cellulose was introduced into this solution under constant stirring and the solution then treated the same as the remaining steps set forth in Example 1.

What is claimed is:

1. A process for the manufacture of cellulosic solutions to be used in the production of threads, filaments, films and the like, which comprises adding hydrogen peroxide to a dilute alkali metal salt solution of the class consisting of alkaline zincate and stannate solutions, mixing cellulose with the solution to form a thick pulp, allowing the cellulose to degrade sufficiently and then cooling the mixture below 0° C. whereupon the cellulose is immediately dissolved.

2. A process for the manufacture of cellulosic solutions to be used in the production of threads, filaments, films and the like, which comprises adding hydrogen peroxide to a dilute alkali metal salt solution of the class consisting of alkaline zincate and stannate solutions, mixing cellulose with the solution to form a thick pulp, allowing the cellulose to degrade sufficiently at a constant temperature and in the presence of nickel sulphate and then cooling the mixture below 0° C. whereupon the cellulose is immediately dissolved.

3. A process for the manufacture of cellulosic solutions to be used in the production of threads, filaments, films and the like, which comprises adding hydrogen peroxide to a dilute alkali metal salt solution of the class consisting of alkaline zincate and stannate solutions, mixing cellulose with the solution to form a thick pulp, allowing the cellulose to degrade sufficiently, destroying the excess hydrogen peroxide with formaldehyde to prevent further degradation of the cellulose, and then cooling the mixture below 0° C. whereupon the cellulose is immediately dissolved.

4. A process for the manufacture of cellulosic solutions to be used in the production of threads, filaments, films and the like, which comprises adding hydrogen peroxide to a dilute alkali metal salt solution of the class consisting of alkaline zincate and stannate solutions, mixing cellulose with the solution to form a thick pulp, allowing the cellulose to degrade sufficiently at a constant temperature and in the presence of nickel sulphate, destroying the excess hydrogen peroxide with formaldehyde to prevent further degradation of the cellulose and then cooling the mixture below 0° C. whereupon the cellulose is immediately dissolved.

5. A process for the manufacture of cellulosic solutions to be used in the production of threads, filaments, films and the like, which comprises adding hydrogen peroxide to a dilute sodium zincate solution, mixing cellulose with the solution to form a thick pulp, allowing the cellulose to degrade sufficiently at a constant temperature and in the presence of nickel sulphate and then cooling the mixture below 0° C. whereupon the cellulose is immediately dissolved.

6. A process for the manufacture of cellulosic solutions to be used in the production of threads, filaments, films and the like, which comprises adding hydrogen peroxide to a dilute sodium zincate solution, mixing cellulose with the solution to form a thick pulp, allowing the cellulose to degrade sufficiently, destroying the excess hydrogen peroxide with formaldehyde to prevent further degradation of the cellulose, and then cooling the mixture below 0° C. whereupon the cellulose is immediately dissolved.

7. A process for the manufacture of cellulosic solutions to be used in the production of threads, filaments, films and the like, which comprises adding hydrogen peroxide to a dilute sodium zincate solution, mixing cellulose with the solu-

tion to form a thick pulp, allowing the cellulose to degrade sufficiently at a constant temperature and in the presence of nickel sulphate, destroying the excess hydrogen peroxide with formaldehyde to prevent further degradation of the cellulose and then cooling the mixture below 0° C. whereupon the cellulose is immediately dissolved.

8. A process for the manufacture of cellulosic solutions to be used in the production of threads, filaments, films and the like, which comprises adding hydrogen peroxide to a dilute sodium zincate solution at approximately 25° C., mixing cellulose with the solution to form a thick pulp, allowing the cellulose to degrade for about 48 hours at the same temperature, cooling the mixture below 0° C. whereupon the cellulose is immediately dissolved and then raising the solution to room temperature in readiness for spinning.

9. A process for the manufacture of cellulosic solutions to be used in the production of threads, filaments, films and the like, which comprises adding nickel sulphate and hydrogen peroxide to a dilute sodium zincate solution at approximately 25° C., mixing cellulose with the solution to form a thick pulp, allowing the cellulose to degrade for about 48 hours at the same temperature, cooling the mixture below 0° C. whereupon the cellulose is immediately dissolved and then raising the solution to room temperature in readiness for spinning.

10. A process for the manufacture of cellulosic solutions to be used in the production of threads, filaments, films and the like, which comprises adding hydrogen peroxide to a dilute sodium zincate solution at approximately 25° C., mixing cellulose with the solution to form a thick pulp, allowing the cellulose to degrade for about 48 hours at the same temperature, adding sufficient formaldehyde to prevent further degradation of the cellulose, cooling the mixture below 0° C. whereupon the cellulose is immediately dissolved and then raising the solution to room temperature in readiness for spinning.

11. A process for the manufacture of cellulosic solutions to be used in the production of threads, filaments, films, and the like, which comprises adding nickel sulphate and hydrogen peroxide to a dilute sodium zincate solution at approximately 25° C., mixing cellulose with the solution to form a thick pulp, allowing the cellulose to degrade for about 48 hours at the same temperature, adding sufficient formaldehyde to prevent further degradation of the cellulose, cooling the mixture below 0° C. whereupon the cellulose is immediately dissolved and then raising the solution to room temperature in readiness for spinning.

AART BUURMAN.

#### REFERENCES CITED

The following references are of record in the file of this patent:

#### UNITED STATES PATENTS

| Number    | Name      | Date           |
|-----------|-----------|----------------|
| 646,799   | Bronnert  | Apr. 3, 1900   |
| 908,754   | Crumiere  | Jan. 5, 1909   |
| 1,279,200 | Wilson    | Sept. 17, 1918 |
| 2,289,085 | Halewijn  | July 7, 1942   |
| 2,322,427 | Edelstein | June 22, 1943  |
| 2,368,527 | Edelstein | Jan. 30, 1945  |

#### FOREIGN PATENTS

| Number     | Country | Date         |
|------------|---------|--------------|
| 37,432     | France  | Feb. 9, 1939 |
| 75 118,836 | Germany | Mar. 7, 1901 |